

Dec. 25, 1928.

1,696,596

C. DANTSIZEN

RESISTANCE UNIT

Filed April 5, 1926

Fig.1.



Fig.2.



Fig.3.



Inventor:  
Christian Dantsizen,  
by *Wm. S. Lint*  
His Attorney.

## UNITED STATES PATENT OFFICE.

CHRISTIAN DANTSZEN, OF SCHENECTADY, NEW YORK, ASSIGNOR TO GENERAL ELECTRIC COMPANY, A CORPORATION OF NEW YORK.

## RESISTANCE UNIT.

Application filed April 5, 1926. Serial No. 98,778.

The present invention relates to conductors of high resistivity and more particularly to such conductors which are commonly employed in connection with vacuum tubes and known as grid leaks. Resistance elements of this type have been made by drawing lines on paper, by spraying or painting porcelain or glass with graphite and by various other well known methods. Such resistances, however, usually have a serious disadvantage in that they vary in conductivity from time to time. The paper resistor, for example, is somewhat unstable, due to the fact that the cellulose fibers are hygroscopic or affected by light, and in the very slight movements of the resistor unit the layer of conducting material is easily disturbed and its conductivity thereby changed. Likewise, when resistance units are made by spraying or painting, it is difficult to obtain uniformity in the value of the resistance.

In accordance with my invention, the resistor comprises an anhydrous material such as a glass rod having an etched surface, and provided at the end portions thereof with a layer of conducting material. Lines are drawn on the etched surface of the glass rod and from end to end thereof with a carbon pencil until enough carbon has been rubbed on to the roughened surface of the glass to provide a resistance element having the desired conductivity. Resistance elements constructed in this manner are practically constant in value and remain so throughout the life of the unit.

The accompanying drawing illustrates in Fig. 1 a glass rod from which sections may be cut to provide the resistance units; Fig. 2 is a perspective view illustrating the method of applying a conducting surface to the glass rod; while Fig. 3 is a cross sectional view illustrating the completed resistor unit.

In carrying my invention into effect, a glass or other suitable insulator rod 1 having a diameter of approximately one-eighth inch is dipped into a solution of acid ammonium fluoride for a period of approximately 30 seconds in order to etch or roughen the surface of the rod. The rod is then washed and dried, and cut into suitable lengths 2, as indicated in Fig. 1. Conductors 3 and 4, which may be made of 20 mils Dumet wire, are then sealed into the opposite ends of each rod 2 and the ends of the rod of the adjacent end portions of the conductors are given surface

conducting coatings, as indicated at 5 and 6. The coatings may comprise, for example, a graphite composition known as "aquadag", and I understand this term to designate suspensions of graphite of colloidal fineness in water. Coatings 5 and 6 are of relatively high conductivity.

The rod 2 is now supported between clips, as indicated at 7 and 8 in Fig. 2. A source of energy, such as a battery, and a milliammeter, neither of which are shown on the drawing, are then connected in series with the wires 3 and 4. While thus connected a graphite or carbon pencil 9 is drawn from end to end of the etched glass rod 2 until sufficient conducting material has been rubbed on to the roughened surface of the glass to give a milliammeter reading corresponding to the quotient of the applied voltage and the desired resistance. The resistance element is then sealed into a glass tube or container 10, as indicated in Fig. 3.

In the use of grid leaks for radio sets, it is important that the resistance element show as little high frequency variation as possible. This property is particularly desirable because variations in the resistance of the grid leak are transmitted through the detector and amplified by the succeeding amplifying tubes thus giving rise to scratching or distortion in the resulting signal. I have found by numerous tests that the type of grid leak which I have described shows little or no high frequency variations and that, as a result, there is practically no distortion in received signals arising from the use of this form of resistive element.

What I claim as new and desire to secure by Letters Patent of the United States is:

1. A method of constructing a resistance unit which comprises etching the surface of a rod of vitreous material, sealing conductors into the ends of the rod, applying a conducting coating to a portion of said conductors and to the ends of said rod, and drawing one or more conducting lines on the roughened vitreous surface to electrically connect said conducting coatings.

2. A conductor comprising a rod of vitreous material having a roughened surface, a pair of wires sealed into opposite ends of the rod, the ends of said rod being provided with a surface layer of conducting material in contact with said wires, said roughened surface being provided with a deposit of

conducting material connecting said surface layer.

3. A conductor comprising a glass rod having an etched surface, a pair of wires sealed into opposite ends of the rod, a surface layer of conducting material on each end of said rod and in contact with said wires, the etched surface of the rod being provided with one or more conducting lines connecting said surface layers.

4. The method of constructing a resistance

unit, which comprises roughening the surface of a rod of vitreous material, sealing conductors into the ends of the rod, applying a conducting coating to a portion of said conductors and to the ends of said rod, and drawing one or more conducting lines on the roughened vitreous surface to electrically connect said conducting coatings. 15

In witness whereof, I have hereunto set my hand this 2nd day of April, 1926.

CHRISTIAN DANTSIZEN.